

## UNITED STATES PATENT OFFICE

2,490,938

## METHOD OF DRYING

James G. Wiegerink, Ridley Park, Pa., assignor to  
 American Viscose Corporation, Wilmington,  
 Del., a corporation of Delaware

No Drawing. Application May 5, 1945,  
 Serial No. 592,269

1 Claim. (Cl. 34—1)

**1**  
 This invention relates to a method of drying packages of fibrous or filamentary material, such as wound packages of fabrics, felts, yarns, tows, slivers and the like, or thick mats of staple fibers. The invention is applicable to the drying of such wound packages or bulky masses of any fibrous material, natural or artificial, such as cotton, silk, rayon, acetate rayon, other cellulose derivatives, nylon, other synthetic resins including polyvinyl chlorides, copolymers of polyvinyl chlorides with acrylonitrile or vinyl acetate, polyvinylidene chlorides, caseins and other proteins, wool, kapok, etc. However, to simplify the description and to illustrate an especially important application of the method, the invention is hereinafter described particularly with reference to regenerated cellulose filaments and staple fibers obtained from viscose or cuprammonium cellulose solutions.

It has heretofore been suggested to apply high frequency induction, either electromagnetically or electrostatically, to heat and dry packages of rayon, such as the annular wound "cakes" of regenerated cellulose filaments as collected in centrifugal spinning buckets, after suitable liquid treatment thereof. The induction heating method has heretofore been suggested in order to overcome the difficulties which arise when using ordinary drying methods, such as currents of heated air, because of the fact that the outer windings of the cake tend to shrink during drying, whereas the inner windings oppose such shrinkage because the drying medium does not penetrate to the inside of the cake sufficiently rapidly to cause it to shrink along with the outer windings. The fact that the inside windings of the cake are allowed free shrinkage, whereas the shrinkage during drying of the outer windings of the cake is opposed, gives rise to strains in the yarns which causes non-uniformity of dyeing of the fabric ultimately produced from the rayon dried by ordinary methods. However, it has been found that the induction method overheats the inside portions of the bulky masses of fibrous material because of the tendency of the vapors developed inside the mass to move to the outer portions thereof. This results in a reversal of the characteristics of the final yarns as compared to those obtained by ordinary drying methods. Such overheating, however, degrades the material composing the fiber, reduces its strength, discolors it and generally affects the fiber properties disadvantageously. The application of a vacuum to assist the evaporation helps this condition somewhat, but is not in itself a complete

**2**  
 answer to the difficulties, since even when a vacuum condition is imposed upon the mass being dried, there is a definite gradient from the middle of the mass to each surface with respect to the moisture content thereof, so that the outer portions of the mass will still contain moisture and need further drying when the windings within the mass have reached bone-dry condition. Continued application of the induction in order to complete the drying of the outer portions of the mass results in injurious effects upon the inner portions of the mass.

In accordance with the present invention, it has been found that drying can be accomplished in an effective economical manner with improved fiber properties in the final dried mass by first heating the mass to be dried by high frequency induction and then completing the drying by ordinary methods, such as by passing heated air or other gaseous medium through the mass. The proportion of moisture removed by the induction applied at the preliminary drying stage may vary widely from a relatively small proportion of about  $\frac{1}{3}$  up to but not over  $\frac{1}{5}$  of the amount of moisture originally present. Then, the drying is completed to the desired moisture content by the circulation of a hot gaseous medium through the mass. By operating in accordance with the present invention it has been found that the straining and non-uniform dyeing properties of the fibers are substantially entirely eliminated, while the danger of overheating parts of the masses is entirely avoided. The surprising and important fact is that the advantages of induction heating in preventing development of strains because of irregular shrinkage effects is not lost by failure to dry the mass completely by that method. These advantages can be preserved and the disadvantages associated with overheating parts of the mass can be overcome merely by removing at least the last fifth of the moisture from the yarn by circulating a hot gaseous medium through the mass without the application of high frequency induction. In addition, the cost of operating in accordance with the invention is intermediate that of high frequency induction drying alone and ordinary circulation of air alone. The present invention also makes it possible to dry larger masses than would be possible with high frequency induction alone as the drying agent.

In speaking of drying, or completing the drying of, rayon or any other of the fibers, it is intended to cover those situations in which a small proportion of moisture is left within the

fibers as well as those in which a condition of so-called "bone dryness" or absolute dryness is reached. Rayon ordinarily has a regain of about 11% moisture, and it is the usual practice to dry originally beyond this point, such as to a content of about 5%, though the precise point to which drying is carried depends upon the particular conditions, such as the size of the package and its density, the point being chosen to assure that all portions of the mass have been carried to a dryness beyond the normal regain.

Wherever percentage moisture content is stated herein, it is based upon the dry weight of the material, such as regenerated cellulose in the case of rayon, so that a mass containing 5% moisture has 5 parts by weight of moisture per 100 parts of dry mass. Moisture is intended in a generic sense to include any liquid.

The preliminary stage of drying in accordance with the present invention may be accomplished by a high frequency coil electromagnetically coupled to the mass to be dried or by a radio frequency oscillator electrostatically coupled through condenser plates to the mass being dried. During the preliminary stage, a vacuum may be applied, or heated air may be circulated through the mass, or a body of air or other gaseous medium having a controlled humidity may be drawn through the mass. The characteristics of the induction field may be varied in conventional manner during the drying, and likewise the humidity of the medium circulated through the mass during the induction stage of heating may be varied as desired, if such a medium is used. Likewise, the gaseous medium circulated through the mass to be dried during the second stage in the absence of high frequency induction may be of any temperature and may have a controlled humidity. However, the advantages of the present invention are generally attainable without the use of controlled humidity and without special care in adjusting the strength of induction field and in varying the temperature of the medium used in the final drying stage. It is for this additional reason that the efficiency of the present invention from a cost standpoint is high.

As stated hereinabove, the high frequency induction heating during the preliminary stage may be continued until all but 1/2 of the moisture originally present is removed from the fibers. This figure is based upon a starting condition in which the regenerated cellulose is in a highly swollen condition as it comes from the wet treatment stages of an artificial filament spinning procedure and before any substantial amount of drying has been performed upon the material. Generally the lower or ultimate limit to which the high frequency induction can be carried in accordance with the invention is about 30% moisture content based on the dry weight of the fibers. This precise figure may vary somewhat, depending upon conditions, such as the size of the package and the characteristics of the high frequency induction field. However, the preferred upper limit of moisture content range which must be reached or passed by the high frequency stage may be defined as that corresponding to the average moisture content of the mass below which portions of the mass do not have surface moisture as distinguished from water of absorption. By "surface moisture" is meant that proportion which is loosely attached to the fiber and is not absorbed in it. When all of the surface moisture has been removed from a portion of the

mass, further application of induction heating causes a heating of the rayon itself in that portion which has lost its surface moisture, and this heating requires a greater transfer of energy per unit of moisture removed than that required merely to remove surface moisture.

The following examples, in which the percent moisture is based on the dry weight of the fibers, illustrate the invention.

10

*Example I*

A batch of cakes of regenerated cellulose were placed in a vacuum chamber and subjected to radio frequency obtained from a 7.5 kilovolt oscillator operating at 25 megacycles. The cakes within the chamber were subjected to a vacuum of about 27 to 28 inches of mercury, and the moisture content was reduced from 190% to 120% in a period of 15 minutes. Then the batch of cakes were passed through a tunnel dryer and air heated at 155° F. was passed through the cakes within the tunnel until only about 5% moisture remained.

*Example II*

15 A batch of high tenacity regenerated cellulose cakes having a moisture content of 130% were dried to a content of 85% moisture between the electrodes of a radio frequency oscillator operated as in Example I, except that no vacuum was used. Again, 15 minutes were required for the induction period and this was followed by air drying at 155° F. to about 5% moisture content.

20

*Example III*

25 A batch of high tenacity regenerated cellulose cakes were dried to a 30% moisture content by radio frequency as in Example II in a period of 30 minutes. This was followed by air drying at 155° F. to 5% moisture content.

30

*Example IV*

35 A batch of regenerated cellulose cakes having 190% moisture content were dried to a moisture content of 50% in a period of 30 minutes while 40 subjected to radio frequency at atmospheric pressure. The cakes were then air dried at 155° F. to 5% moisture.

45

*Example V*

50 Cakes of high tenacity regenerated cellulose yarns were continuously conveyed by means of a belt in sequence through a chamber containing electrodes connected to a radio frequency oscillator disposed on opposite sides of the belt and 55 then through a chamber in which air heated to 155° F. was circulated. The speed of the belt was so adjusted with respect to the distinct heating stages that the cakes took a period of approximately 20 minutes in passing between the radio 60 frequency electrodes, during which they were dried to a 60% moisture content from an initial 130% moisture content and during the subsequent stage took a period of about 20 hours through the air drying tunnel, during which their 65 moisture content was reduced to 5%.

70

*Example VI*

75 A cake of 150 denier 40 filament delustered regenerated cellulose yarn having a moisture content of 190% was dried to a moisture content of 100% by an electromagnetic induction coil. Then air at 135° F. was circulated through the cake until a moisture content of 5% was attained.

The invention is applicable equally as well to 75 batch and continuous handling methods. This

is a special advantage derived from the fact that the present method is not dependent upon the use of a vacuum in order to obtain fibers of improved quality. One advantageous embodiment involves the continuous passage of a belt preferably permeable to vapor carrying the masses to be dried, such as the rayon cakes, at a constant linear speed through a long tunnel, in the first portion of which electrodes may be disposed on opposite sides of the belt or above and below the belt, or coils may be provided to encircle the belt and the last portion of the tunnel is merely provided with conventional means for circulating heated air through the cakes upon the belt. Alternatively other conveying means, such as chain-driven rods may be used for supporting the masses to be dried. The exhaust steam from the powerhouse used for generating the electrical current used in the first stage of the heating, 20 may be used for heating the air in the second stage of the tunnel. Since the preliminary drying is done by means of high frequency induction, and since that stage prevents later development of strains due to irregular shrinkage, the 25 final stage of drying by ordinary means, such as circulation of heated air, may be done more rapidly than is ordinarily the case in conventional tunnel dryers using heated air or other gaseous medium. Thus whereas temperatures 30 of 140 to 155° F. are the conventional ones used, the final drying stage in accordance with this invention may involve air heated to 100° F. up to as high as 200° F. without encountering trouble with dyeing and other irregular effects upon the 35 fiber characteristics.

It is to be understood that changes and variations may be made without departing from the

spirit and scope of the invention as defined by the appended claim.

I claim:

The method of drying a water-moist annular wound package of artificial filaments of regenerated cellulose containing water of absorption and surface moisture resulting from the wet treatment of an artificial filament-spinning procedure comprising the steps of applying high frequency induction at atmospheric pressure to heat the mass internally to vaporize and thereby effect removal of moisture until  $\frac{1}{3}$  to  $\frac{1}{5}$  of the initial moisture content has been removed, interrupting the induction heating before the moisture content of the package has been reduced below one-fifth the initial content, and subsequently removing the remaining moisture by circulation of a heated gaseous medium with respect to the package.

JAMES G. WIEGERINK.

#### REFERENCES CITED

The following references are of record in the file of this patent:

#### UNITED STATES PATENTS

| Number    | Name         | Date          |
|-----------|--------------|---------------|
| 2,042,145 | Darrah       | May 26, 1936  |
| 2,231,457 | Stephen      | Feb. 11, 1941 |
| 2,325,652 | Bierwirth    | Aug. 3, 1943  |
| 2,403,800 | Hoyler       | July 9, 1946  |
| 2,421,334 | Kline et al. | May 27, 1947  |
| 2,428,615 | Brown        | Oct. 7, 1947  |

#### OTHER REFERENCES

"Drying and Laminating by Radio Frequency," by George F. Russell, in "The Timberman," August 1944 issue, pages 38, 40, 42.